

Aug. 1, 1961

H. A. TOULMIN, JR

2,994,297

APPARATUS FOR MAKING MOLDS BY GAS PLATING

Filed Aug. 18, 1958

2 Sheets-Sheet 1



Fig. 1



Fig. 2



Fig. 3

INVENTOR  
HARRY A. TOULMIN, JR.

BY *Toulmin & Toulmin*

ATTORNEYS

Aug. 1, 1961

H. A. TOULMIN, JR

2,994,297

APPARATUS FOR MAKING MOLDS BY GAS PLATING

Filed Aug. 18, 1958

2 Sheets-Sheet 2



*Fig. 4*



*Fig. 5*



*Fig. 6*



*Fig. 7*



*Fig. 8*



*Fig. 9*

INVENTOR  
HARRY A. TOULMIN, JR.

*Fig. 10*

BY *Toulmin & Toulmin*

ATTORNEYS

# United States Patent Office

2,994,297  
Patented Aug. 1, 1961

1

2,994,297

## APPARATUS FOR MAKING MOLDS BY GAS PLATING

Harry A. Toulmin, Jr., Dayton, Ohio, assignor, by mesne assignments, to Union Carbide Corporation, New York, N.Y., a corporation of New York

Filed Aug. 18, 1958, Ser. No. 755,603  
4 Claims. (Cl. 118—48)

This invention relates to apparatus and methods for gas plating. More particularly, the invention is concerned with gas plating forming dies, and especially the plating of metal onto a die forming surface.

Present methods for producing forming dies are costly due to the large amount of hand labor and machining involved. It has been proposed to use plastic dies but their wear resistance is low. Metal sprayed dies are subject to distortion under shock forces and are relatively fragile. Attempts to electroform dies free from stress and resulting distortion have not been achieved with any degree of success.

This invention overcomes these difficulties for all practical purposes and provides an apparatus and method for making forming dies by gas plating.

After carrying out a large number of experimental tests it has been found that in the making of such forming dies, the same may be made by gas plating metal onto a mold having the contour of the desired die shape. A suitable mold is made of gypsum admixed with powdered metal, such as aluminum. Molds also may be made of resins, particularly epoxy resins, and which have been cured to form a thermoset resin body. The pre-shaped mold surfaces are then gas plated to produce forming dies of any desired shape. Dies of very large area and never before attempted by conventional methods have been successfully produced in accordance with this invention.

The gas plating of the mold surface to produce the die may be carried out using various type molds but that found to be very satisfactory was composed of gypsum having powdered aluminum admixed therein in proportions of approximately 50 parts metal to 50 parts gypsum.

In the instant application, the invention will be described with more particularity with respect to the production of forming dies using nickel carbonyl as a gas plating agent. Other suitable gaseous metal bearing compounds may be used where desired, such as chromium carbonyl, molybdenum carbonyl, and the like.

These and other objects and advantages will become apparent from the following description taken in conjunction with the drawings, and wherein—

FIGURE 1 shows in cross section a broken away portion of a mold for forming the die and which mold comprises a series of spaced coils for heating the inner surface of the mold;

FIGURE 2 is a view in elevation of the die portion shown in FIGURE 1;

FIGURE 3 is a view partly in cross section and illustrating the use of the mold structure shown in FIGURE 1;

FIGURE 4 is a fragmentary detailed cross section illustrating a heating element and wherein the same comprises a solid rod or core heated with a coil;

FIGURE 5 is a similar fragmentary cross sectional view as in FIGURE 4 and illustrating a closed top tube through which heated fluid is circulated for heating the mold surface to be gas plated;

FIGURE 6 is a similar fragmentary view as in FIGURE 4, and wherein the rod or solid heating coil element comprises a hammer head portion for extending the heat along the surface portion of the mold which is to be gas plated;

2

FIGURE 7 is a similar cross sectional view of the fragmentary section of the mold and wherein an open tube is used through which heated air is circulated and wherein the upper ends of the tubes are connected with a common channel beneath the surface portion of the mold to be gas plated;

FIGURE 8 is a fragmentary portion of a mold shown in section, and wherein spaced heater coils are arranged in a plane closely adjacent the surface of the mold surface to be gas plated for heating the mold surface for effecting uniform gas plating of metal thereon;

FIGURE 9 is a view in elevation of FIGURE 8, and illustrating the arrangement of heating coils in the mold; and

FIGURE 10 is a fragmentary sectional view of a mold illustrating the use of a tubular structure which is arranged to be heated by a surrounding hollow coil which is in the form of a tube through which heated fluid is circulated for heating the surface portion of the mold to be gas plated.

In the drawings, in FIGURE 1 a plastic mold 11 is shown and which may be composed of gypsum and powdered metal as aforementioned. The surface portion of the mold 12 is of a contour shape to form the die plate 13 and which is produced upon deposition of metal thereon by gas plating.

To heat the die surface portion 13 there is arranged within the body of the mold 11 spaced heating coils 14, which coils are disposed about the tubular opening 15. The tubes 15 extend upwardly and terminate adjacent the die forming surface as at 16. Electrical heating coils 14 are made of the usual resistant material, such as Ni-chrome, and when electrically connected heat the air in the tubes 14 so that they, in turn, heat the mold surface portion 18 at the top of the tubes. In this manner the die forming surface 13 is uniformly heated to the proper temperature whereby gas plating may be efficaciously carried out.

In FIGURE 3, a gas plating chamber 20 is illustrated, and which is arranged over the mold surface 11. The gas plating chamber 20 is provided with an inlet opening 21 and an outlet opening 22 for receiving and discharging gaseous metal bearing compound which is circulated through the gas plating chamber. Heated air is forced upward through the tubes as illustrated by the arrows in FIGURE 3, while the heating coils are connected so that the mold surface portion 18 is heated uniformly to a temperature high enough to thermally decompose the gaseous metal compound, e.g., nickel carbonyl or other metal bearing compound or mixture thereof, which is circulated or conducted into the chamber 20 and in contact with the heated surface 18 and produce the forming die of metal deposited thereby as at 23.

In the modified structure illustrated in FIGURE 4, the mold 25 is equipped with solid rod 26 such as may be made of copper, steel, or the like, and which rods are heated by electrical resistance coils 27 arranged thereabout and connected to a suitable source of electricity. The rods when thus heated convey heat to the surface portion 28 of the mold so as to uniformly heat the area during the gas plating of the metal onto this surface portion to thus form the die of gas plated metal.

In FIGURE 5 the modification illustrated shows a mold 30 having tubes 31 through which heated fluid such as air or liquid is pumped by means of smaller tubes 32 which extend into the larger tube 31. The hot fluid is conveyed to the die-forming surface portion of the mold 34 which is to be uniformly heated and receives the gas plated metal deposit for forming the die.

In FIGURE 6 a similar mold portion is shown at 35

and in which the heat is supplied to the mold surface portion 36 by hammer-headed solid rods 37. The rods which are made of copper, iron, steel or the like, are heated by the surrounding electrical resistance coils 38.

Similarly in FIGURE 7, a mold 40 comprises hollow interconnected tubes 41 which extend upward through the body of the mold and communicate with a common channel 42 disposed immediately beneath the mold surface portion 43 which is uniformly heated and subjected to gas plating. The fluid is circulated through the tubes as illustrated by the arrows in FIGURE 7, and the tubes are heated by resistance coils 44.

FIGURE 8 illustrates a similar mold 45 and wherein the surface portion of the mold 46 which is to be heated to effect the gas plating comprises spaced electrical heating resistance coils, the same being disposed immediately beneath the mold surface 46, as illustrated in FIGURE 9.

In FIGURE 10, a mold 50 is shown and wherein the mold die-forming surface portion 51, and which is to be gas plated in the production of the forming die, is heated by an open tube 52 extending upwardly and adjacent the surface 51. The tubes 52 are heated by means of surrounding fluid heated coils 53 and through which heated fluid such as water, mercury or the like is circulated.

In the making of the dies use may be made of different mold shapes, the composition of which must be such as to provide a stable mold at the temperature of gas plating.

A suitable mold composition from which a shaped mold may be made comprises the following constituents by weight:

| Parts by weight                           |   |
|-------------------------------------------|---|
| Hydrated calcium sulfate (gypsum)         | 2 |
| Aluminum metal powder (325 mesh or finer) | 2 |
| Water                                     | 1 |

Aluminum metal particles provide the desired coefficient of expansion of the mold. This prevents distortion and dimensional changes during gas plating and production of the forming die. The gypsum enhances the thermal stability of the mold and provides a strong shock resistant mold.

In place of a gypsum-aluminum metal mold the same mold shape may be made of gypsum and admixed with glass fibers for a portion or all of the metal. In place of aluminum, iron metal powder or the like metal may be substituted.

A suitable resin mold is made using epoxy resin with

ing plate to make a completed die. This procedure is repeated to form the complementary die or lower die.

The gas plating is carried out in the conventional manner at ordinary atmospheric pressure, and using a carrier gas such as carbon dioxide. The gas plating rate is proportional to the rate of evolution of carbon monoxide employing metal carbonyls. A satisfactory plating rate results when using nickel carbonyl at temperatures between 375° F. and 400° F. Gas plating of the mold surfaces to form the dies is preferably carried out as a continuous gas plating operation until the desired thickness of die plate is obtained to avoid the formation of laminations in the die plate structure. The heating elements of the mold are controlled so as to heat the mold surface portion which is to receive the metal deposit to a temperature high enough to cause thermal decomposition of the gaseous metal compound, e.g., nickel carbonyl, and deposition of the nickel metal to produce the die.

In carrying out the gas plating it was found that an important factor in the attainment of proper plating temperatures and high gas plating efficiency was effected by providing the heating coil arrangement and pattern within the mold in accordance with this invention. The thermal conductivity of the mold substrate is relatively poor, however, by providing internal mold heating means closely adjacent the mold surface portion which is to receive the metal deposit as illustrated and described, an excellent detail production of the die contour shape is obtained.

In practicing the gas plating method to form dies of nickel metal, for example, nickel carbonyl and carbon dioxide carrier gas is introduced on a parallel flow from separate vaporizers which is connected to a common manifold communicating with the gas plating chamber. Liquid nickel carbonyl is connected to a separate vaporizer from which the gaseous nickel carbonyl flows and is admixed with carbon dioxide carrier in the manifold. This arrangement minimizes possible interruptions of the gas flow to the gas plating chamber which is desirable to permit continuous gas plating.

A die face area of approximately 656 square inches was gas plated with nickel metal as described to a thickness of about 1/4 inch to 1/2 inch. The average consumption of nickel carbonyl was 12 3/4 pounds per hour.

The following table shows the results of gas plating runs made using both epoxy resin and aluminum-gypsum mold compositions.

Table I

| Run | Mold            | Mold Temp., °F. | Carrier Gas     | Plating Gas     | Nickel Carbonyl flow rate, cc./mm. | CO <sub>2</sub> flow rate (cu. ft./hr. at 160° F.) | Plating Time, hrs. | Remarks                                                   |
|-----|-----------------|-----------------|-----------------|-----------------|------------------------------------|----------------------------------------------------|--------------------|-----------------------------------------------------------|
| 1   | Aluminum Gypsum | 385             | CO <sub>2</sub> | Nickel Carbonyl | 7.2                                | 12                                                 | 21 1/4             | Excellent detail and ductile metal die.                   |
| 2   | Epoxy Resin     | 405             | CO <sub>2</sub> | do              | 7.1                                | 12                                                 | 17 1/2             | Similar to gypsum mold but darker shade of metal deposit. |

or without the addition of fillers such as metal or glass powders. An example of an epoxy resin for forming the mold shape, and which will withstand gas plating with nickel carbonyl is made by admixing (in parts by weight) 57 parts of bisphenol-A with 195 parts diglycid ether, 46.5 parts aniline and 15 parts of sodium hydroxide, the mixture being heated and reacted at 212° F. for an hour to convert the mass into an infusible resin product.

In the producing of the gas plated forming dies, the following steps are carried out (1) shape the mold surface to the desired die contour; (2) gas plate the mold contour surface to deposit a uniform thickness of metal, e.g., nickel, to produce the die structure; (3) strip the metal plate from the mold surface; and (4) add a back-

Dies formed in accordance with the invention are composed of substantially pure metal and exhibit high tensile strength, excellent ductility, high degree of hardness, and are dense metal structures free of internal stresses.

One of the great advantages of the invention is that the mold is reinforced by the heating tubes or rod means embedded in the body of the molds. This reinforced mold structure prevents distortion and compression of the mold while being subject to gas plating. The spaced heating means also evenly distributes the heat both through the convection of the heated air or fluid as well as by radiation. In this manner by regulating the heat applied to the spaced heating elements, accurate control of the temperature of the mold can be obtained. This is important to prevent a fire hazard where the mold com-

pries finely divided metal particles dispersed throughout the mold and which particles are pyrofic. Metal particles such as the non-ferrous as well as ferrous, e.g. stainless steel may be used to vary the heat conductivity and heat conditions of this mold whereby different heat requirements for gas plating with different metal bearing compounds can be readily satisfied.

Gas plating production of dies permits the making of die working surfaces of accurate and fine detail contour shapes. Moreover, complex areas and contours can be uniformly gas plated with metal at high rates not possible by conventional methods.

It will be understood that while there have been described and illustrated certain specific embodiments of the invention, it is not intended thereby to limit the same thereto inasmuch as the invention is readily susceptible to various modifications, and the use of different metal bearing gas plating compounds, and substitutions of materials, as may be made by those skilled in the art all of which come within the scope of the invention, and as set out in the appended claims.

What is claimed is:

1. An apparatus for making metal forming dies by gas plating, said apparatus comprising a mold composed of gypsum and aluminum metal particles and having a surface portion shaped in conformity with the contour shape of the metal forming die to be made, said mold including hollow fluid heated tubes spacedly disposed in the body of said mold and terminating at one end closely adjacent said mold surface for heating said mold surface portion to a temperature high enough to effect the gas plating of metal on said mold surface portion to produce the metal forming die.

2. An apparatus for making metal forming dies by gas plating, said apparatus comprising a mold composed of gypsum and aluminum metal particles and having a surface portion shaped in conformity with the contour shape

of the metal forming die to be made, said mold including heated solid rods spacedly disposed in the body of said mold and terminating at one end closely adjacent said mold surface for heating said mold surface portion to a temperature high enough to effect the gas plating of metal on said mold surface portion to produce the metal forming die.

3. An apparatus for making metal forming dies by gas plating, said apparatus comprising a mold composed of gypsum and aluminum metal particles and having a surface portion shaped in conformity with the contour shape of the metal forming die to be made, said mold including hollow tubes disposed in the body of said mold through which heated fluid is circulated, said tubes being arranged for heating said mold surface portion to a temperature high enough to effect the gas plating of metal on said mold surface portion to produce the metal forming die.

4. An apparatus for making metal forming dies by gas plating, said apparatus comprising a mold composed of gypsum and aluminum metal particles having a surface portion shaped in conformity with the contour shape of the metal forming die to be made, said mold comprising electrical heating coils disposed in the body of said mold and beneath the mold surface for heating said mold surface portion to a temperature high enough to effect the gas plating of metal on said mold surface portion to produce the metal forming die.

References Cited in the file of this patent

UNITED STATES PATENTS

|           |            |       |                |
|-----------|------------|-------|----------------|
| 1,950,605 | Fitzgerald | ----- | Mar. 13, 1934  |
| 2,256,247 | Groehn     | ----- | Sept. 16, 1941 |
| 2,333,534 | Lang       | ----- | Nov. 2, 1943   |
| 2,602,033 | Lander     | ----- | July 1, 1952   |

FOREIGN PATENTS

|        |               |       |      |
|--------|---------------|-------|------|
| 21,025 | Great Britain | ----- | 1890 |
|--------|---------------|-------|------|